

## UNITED STATES PATENT OFFICE

2,036,962

## METHOD FOR PRODUCTION OF FIRMLY ADHERING GALVANIC COATINGS ON ALUMINUM AND ALUMINUM ALLOYS

Johannes Fischer, Berlin-Charlottenburg, Germany, assignor to Siemens & Halske, Aktiengesellschaft, Siemensstadt, near Berlin, Germany, a corporation of Germany

No Drawing. Application February 1, 1934, Serial No. 709,349. In Germany February 15, 1933

2 Claims. (Cl. 204—3)

This invention relates to a method for production of firmly adhering galvanic coatings on aluminum and aluminum alloys.

According to prior proposals one produces firmly adhering coatings on aluminum and aluminum alloys by first producing an oxide layer by anodic treatment of the metals preferably in baths containing chromic acid, then detaching partially the so formed oxide layer by cathodic treatment in alkaline baths containing salts of heavy metals, e. g. copper and so simultaneously forming an intermediate copper layer of interrupted structure, finally plating the so prepared body. It is also known to use alternating current and an alkaline bath for the production of the artificial oxide layer.

It has now been discovered that it is possible to get metal coatings of particularly firm adherence on aluminum and its alloys by treating the bodies in a phosphoric acid solution with direct or alternating current to produce an oxide film on their surfaces.

The concentration of the phosphoric acid solution may vary within wide limits, the use of concentrations between one and ten percent being advantageous. It is further advantageous, but not necessary to keep the temperature of the bath constant at forty to fifty degrees centigrade. Lower temperatures are used if the aluminum alloys contain greater percentages of heavy metals.

After treating the bodies in the phosphoric acid bath one continues the process according to the method hereinbefore described, i. e. one makes the oxidized articles cathodes in an alkaline bath containing copper or brass whereby a part of the oxide layer disappears and a small quantity of copper or brass is simultaneously precipitated, and finally plates the body so prepared.

In its broad aspects my invention comprises producing an oxide layer on an article of aluminum or of an aluminum alloy by electrical treatment thereof in an aqueous phosphoric acid bath, the concentration of the acid, temperature of the bath, duration of the treatment and other conditions being so correlated and controlled as to form an adherent oxide layer, which layer is sufficiently porous to receive an adherent metallic flash coating in an alkaline plating bath, thereupon flash-coating said article over the resulting oxide layer in an alkaline electroplating bath, and then finish-plating said article. The oxide layer produced in my process should correspond substantially in character to that produced by the specific example which follows.

In an illustrative example of my process an aluminum article was put into a three percent bath of phosphoric acid at about forty degrees centigrade. This article was made an anode. The initial current reached a value of about 60 amperes. This current decreased within a few seconds to about twenty amperes, the voltage increasing to ninety or hundred volts simultaneously. The article having been so oxidized during five minutes was then carefully rinsed and put into an alkaline bath containing copper and zinc salts. It was there flash-coated with brass as an intermediate metal by being made a cathode at a voltage of five volts. Sufficient brass was precipitated after five minutes treating. After this treatment an article can be finish-plated in any of the usual metal plating baths.

In the second stage of my process in which an intermediate metallic coating is produced, any one of the usual alkaline degreasing baths may be employed with the addition to said bath of the usual metallic salts required for producing the desired intermediate coatings.

There are some important advantages of the method according to the invention enumerated above:

(1) In case of insufficient rinsing the phosphoric acid does not impair the alkaline bath as does the chromic acid. Chromic acid interferes with the second stage of the coating process as it affects generally all galvanic processes.

(2) The handling of chromic acid is avoided with its attendant risks to the health of the workmen.

(3) A great number of different alloys, for example, magnesium containing alloys, may be oxidized in phosphoric acid baths which is often impossible if chromic acid is used as electrolyte or if the oxidation process is conducted with alternating current in a solution of sodium carbonate.

(4) The process may be operated with direct or alternating current in the same bath at will.

(5) There is no strict rule for the duration of the oxidation period. Using chromic acid the oxide layer after a fixed period will become so thick that it cannot be detached by the cathodic treatment in the alkaline bath. Using phosphoric acid the time of treating is much less critical. For example it is possible to allow the articles to stay in the phosphoric acid bath during a whole hour or more without deterioration of the past precipitated oxide coating. This independence upon the time of treating is very important in

commercial practice because it simplifies the control of the process.

Further it was found that the efficacy of the oxide layer is dependent upon its porosity. If its thickness becomes so great that current cannot pass at all, the oxide layer—as explained hereinbefore—cannot further form a suitable base for the superimposed copper or brass coating, because it is very difficult to partially detach such oxide layers in the alkaline bath.

10 Three factors must be carefully controlled in the production of porous layers:

- (a) duration of oxidation,
- (b) temperature and
- (c) concentration of the electrolyte.

15 The importance of the duration has been mentioned hereinbefore. The temperature of the electrolyte has also great influence on the character of the layer, which becomes more porous at higher temperatures while being difficult to produce in such porous form at lower temperatures. Therefore the duration of oxidation also may be varied within wider limits at higher temperatures than at lower ones.

20 25 Similarly porous layers are more easily attained at higher than at lower concentrations of the electrolyte.

It is known to form oxide layers on aluminum electrodes for the purpose of polarization. It is 30 furthermore well known to treat aluminum bodies with direct or alternating current in soda or barium peroxide solutions containing small quantities of phosphoric acid for producing insulating layers on aluminum. But these known methods are comparable only with the first stage of the process according to this invention which is characterized by the unity of its three stages and serves for quite different purposes.

What I claim is:

1. In the plating of firmly adherent metallic coatings on aluminum and aluminum alloys, the process which comprises producing an oxide layer on such an article by electrical treatment thereof in an aqueous phosphoric acid bath, the concentration of the acid, temperature of the bath, duration of the treatment and other conditions being so correlated and controlled as to 10 form an adherent oxide layer, which layer is sufficiently porous to receive an adherent metallic flash coating in an alkaline plating bath, thereupon flash-coating said article over the resulting oxide layer in an alkaline electroplating bath, 15 and then finish-plating said article.

2. The process of claim 1, wherein the conditions of the treatment in the phosphoric acid bath are so correlated as to correspond substantially to a treatment for about five minutes in 20 an aqueous bath of phosphoric acid of about 3 per cent concentration, maintained at a temperature ranging from about 40 to 50° C., and with a voltage increasing during treatment to a value of from about 90 to 100 volts.

JOHANNES FISCHER.